

# UNITED STATES PATENT OFFICE.

OSKAR KALTWASSER, OF BERLIN, AND HANS OEHORN, OF BERLIN-CHARLOTTENBURG, GERMANY, ASSIGNORS TO ACTIEN GESELLSCHAFT FÜR ANILIN FABRIKATION, OF BERLIN, GERMANY.

## PROCESS FOR DYEING SKINS, HAIRS, AND THE LIKE.

1,416,646.

Specification of Letters Patent. Patented May 16, 1922.

No Drawing.

Application filed December 7, 1921. Serial No. 520,696.

*To all whom it may concern:*

Be it known that we, OSKAR KALTWASSER and HANS OEHORN, the first a citizen of the German Republic, the second owns no citizenship, residing at Berlin, Germany, and Berlin-Charlottenburg, Germany, our P. O. address being Urbanstr. 178, Berlin, Germany, and Mommsenstr. 13, Berlin-Charlottenburg, Germany, have invented certain new and useful Improvements in Processes for Dyeing Skins, Hairs, and the like, of which the following is a specification.

We have found that the 5-nitro-2-amino-1-oxy-derivatives of the benzene series are excellently fitted for dyeing skins, hairs and the like mordanted or not in the presence of a suitable oxydizing agent, such as hydrogen-peroxide. Thus are obtained yellow to brown dyeings of a great intensity and an excellent fastness to light.

The following example illustrates the invention, without limiting it.

The skin to be dyed is washed for about an hour in water containing 10 to 20 grams of calcined sodium carbonate per liter, well rinsed and then dyed at ordinary temperature during 3 to 5 hours in a bath which contains per liter 2 grams of 5-nitro-2-amino-1-oxybenzene, 2 grams of ammonia of 25% strength and 30 grams of hydrogen peroxide of 3% strength. Then the skin is

rinsed and worked up as usual. A clear yellow tint is the result.

On skins previously mordanted with iron-mordants yellow tints are also obtained; on skins mordanted with chromium- or copper-mordants brown dyeings are produced. In like manner substitution products of 5-nitro-2-amino-1-oxybenzene, such as its homologues, may be employed.

Having now described our invention and the manner in which it may be performed what we claim is—

1. The herein-described process for dyeing skins, hairs and like materials which comprises treating the material in the presence of a suitable oxidizing agent in a bath containing a 5-nitro-2-amino-1-oxy derivative of the benzene series.

2. The herein-described process for dyeing skins, hairs and like materials which comprises treating the mordanted material in the presence of a suitable oxidizing agent in a bath containing 5-nitro-2-amino-1-oxybenzene.

In testimony whereof we affix our signatures in presence of two witnesses.

Dr. Phil. OSKAR KALTWASSER.  
HANS OEHORN.

Witnesses:

HERMANN KIRCHHOFF,  
FRITZ SCHILK.